

April 13, 1937.

M. W. KROLL

2,077,332

PROCESS OF AND APPARATUS FOR AMALGAMATING AND SEPARATING METALS

Filed Feb. 19, 1934

3 Sheets-Sheet 1



Martin W. Kroll, INVENTOR  
BY Victor J. Granatello.

ATTORNEYS

April 13, 1937.

M. W. KROLL

2,077,332

# PROCESS OF AND APPARATUS FOR AMALGAMATING AND SEPARATING METALS

Filed Feb. 19, 1934

3 Sheets-Sheet 2



Pl. 2.

*Martin W. Kroll* INVENTOR  
BY *Victor J. Evans & Co.*

ATTORNEYS

April 13, 1937.

M. W. KROLL

2,077,332

PROCESS OF AND APPARATUS FOR AMALGAMATING AND SEPARATING METALS

Filed Feb. 19, 1934

3 Sheets-Sheet 3

*Fig. 4.*



*Fig. 3.*



*Martin W. Kroll, Inventor*  
BY *Victor J. Evans & Co.*

ATTORNEYS

## UNITED STATES PATENT OFFICE

2,077,332

## PROCESS OF AND APPARATUS FOR AMALGAMATING AND SEPARATING METALS

Martin W. Krell, Billings, Mont.

Application February 19, 1934. Serial No. 712,026

1 Claim. (Cl. 204—15)

The invention relates to a process of and apparatus for amalgamating and separating metals.

The primary aim of the present invention is to provide a process of and apparatus of this character wherein in their use for the purpose of extracting metals from finely ground ore, they will enable the finely ground ore to mix with the solution in the proper ratio to keep the mass in a fluid or liquid state and the resultant pulp comprising the pulverized ore and solution will be sustained in a state of agitation so that all ore particles will be suspended to the extent that no settling will occur at the bottom of the vat, the rate of agitation being, of course, varied in accordance with the specific gravity of the material under treatment.

Another object of the invention is the provision of a process of and apparatus of the kind specified, wherein the agitation which is necessary to keep the mineral particles in the solution suspended may be produced by utilizing a down-draft propeller, mechanically driven at the proper speed, and in some instances, it may be found necessary or beneficial to utilize the propeller for disintegration of material, this being had by perforating the propeller blades. The disintegration action is found especially beneficial in freeing extremely fine gold from clay, the action of the propeller producing a constantly moving stream of material with a downward motion, while it is also possible to utilize an electric current of the proper voltage, current density and frequency for the production of electrical precipitation, separation or amalgamation of the metallic particles while suspended and under agitation, these particles being deposited on a cathode or electrical conductor plate disposed in the bottom of a vat and of such material or composition as to produce the desired result in connection with the mineral under treatment.

A further object of the invention is the provision of a process of and apparatus for amalgamating or extracting ores or metals, wherein the solution used in connection with the ore under treatment be of such a chemical nature as to produce a condition which will aid in bringing about extraction of the desired metals and the electrical resistance of the solution controlled by the addition of salts, acid or alkali in the correct proportions to bring about a desired state of conductivity in the solution and also that will, in many instances, produce chemical changes in the material under treatment so that the time of treatment, the cost of electric current and the percentage of abstraction obtainable can be made

more favorable. In some instances, the use of a chemical reagent makes it possible to so change the chemical composition of the material under treatment that although it may be partially or entirely refractory in its original state, the alteration in the nature of the material will enable the same to yield to the process.

In the accompanying drawings:

Figure 1 is a side elevation of the apparatus constructed in conformity with the invention and employed in carrying out the process of amalgamation and separation of ores.

Figure 2 is a vertical longitudinal sectional view thereof.

Figure 3 is a vertical transverse sectional view taken on the line 3—3 of Figure 2 looking in the direction of the arrows.

Figure 4 is a view similar to Figure 3 showing a slight modification of the apparatus.

Similar reference characters indicate corresponding parts throughout the several views in the drawings.

Referring to the drawings in detail, particularly Figures 1 to 3 inclusive, the apparatus for the amalgamation and separation of ores, as constructed in conformity with the present invention, comprises a substantially V-shaped agitating vat A which includes the opposite vertically disposed spaced parallel side walls 5, these being joined in any suitable manner with upwardly divergent spaced end walls 6 for a hopper formation of the vat. Beneath the said vat is a combined settling and filtering vat 1, the same being divided at an intermediate point by a vertical partition 8 to provide the settling chamber 9 and the filtering chamber 10, respectively, the partition being formed with a filtering screen 11 of any approved construction, so that the liquid or fluid passing from one chamber to the other will be subjected to the filtering action of the filter 11, as will be obvious.

Rising from the vat 1 at one side of the vat A are suitable supports 12 for a platform 13 on which is arranged a pump 14 of the motor or hand driven type having the lift pipe or cylinder 15 which extends within the chamber 9, so that its contents can be returned to the vat A, the delivery of the liquid from the pump 14 into the vat A being had through the discharge spout 16 of said pump 14.

Mounted in suitable bearings 17 arranged near the top of the vat A, at one end thereof, is the shaft 18 of an agitator having the propeller blades 19 of the form to effect a down draft within the said vat A, the shaft 18 of the agitator being

5

10

15

20

25

30

35

40

45

50

55

55

disposed at the same inclination of the end walls 6 of the vat A next thereto. Suitably supported upon the vat A is an electric motor 20 which, through the pulleys 21 and belt 22, respectively, has connection with the shaft 18 of the agitator so that the latter will be driven directly from this motor.

Located at the lowermost point of the vat A is a mercury cathode 23 having the metallic plate 24 constituting a bottom to the vat A and this plate is fitted with a mercurial drain 25, while carried by the end walls 6 next to the shaft 18 of the agitator is an anode 26, both 23 and 26 being connected by the negative and positive current leads 27 and 28, respectively, to a direct current supply (not shown), the level of the mercurial column of the cathode 23 being indicated at 29 within the vat A.

In the process for the extraction of metals by electrical amalgamation and separation, the apparatus is employed and for the purpose of extracting metals from finely ground ore, the finely ground ore is mixed with a solution in the proper ratio to keep the mass in a fluid or liquid state and such ore and the solution is admitted into the vat A so that the pulp comprising the pulverized ore and solution will be mixed and kept in a state of agitation by the agitator, whereby all ore particles will be maintained in suspension to the extent that no settling will occur at the bottom of the vat A. Of course, the rate of agitation is varied in conformity with the specific gravity of the material under treatment and such agitation is essential to keep the mineral particles in the solution suspended, the agitation being in a downward direction, the propeller blades 19 being located beneath the level of the solution or the mixture as contained within the vat A and the agitator producing a constantly moving stream of material with a downward motion so as to bring about an intimate contact of all particles suspended with the bottom of the vat.

By using the down draft, force of gravity is utilized in helping to bring all particles suspended in contact with the bottom of the vat A and in combination therewith it is possible to use electric current to assure electrical precipitation, separation or amalgamation of the metallic particles suspended in the vat A at the time of agitation and to deposit these mineral particles on the cathode 23 located at the lowermost point of the vat A. The anode 26 for conducting the electric current is so placed in the vat that the exposed area in contact with the solution may be varied to meet specific requirements. Furthermore, the distance of air gap between the anode and the cathode may be varied by the adjustable members 30 for regulating current density, and the material comprising the anode and the cathode is to be of a composition which will prevent excessive disintegration of the anode, the cathode material being determined by the material to be treated.

The electrical resistance of the solution as used within the vat A is controlled by the addition of salts, acid or alkalies in the correct proportions to bring about a desired state of conductivity in the solution, as well as in many instances to produce chemical changes in the material under treatment, so that the time of treatment, the cost of electrical current and the percentage of extraction obtainable can be made more favorable.

It is also possible to bring about a complete

extraction of the desired metal from a continuous flow through the vat by the use of a chemical reagent, the incoming feed of pulp to the vat A and the discharge rate being regulated in accordance with the time required for satisfactory extraction from the material under treatment.

In one side wall 5 of the vat A is arranged a gate valve 31, the same being disposed approximately one foot above the extreme bottom of the said vat and this valve being utilized to facilitate discharging the pulp after satisfactory extraction of the metals in the material under treatment. The material in the vat A is kept in a state of agitation during the period of time required for discharging the tailings and the fresh solution being pumped into the top of the vat at the same rate that the solution is drained off through the discharge valve 31, the pump 14 being actuated to deliver the fresh solution into the vat A. The valve 31 has connected thereto a flexible pipe 32 for the discharge from the vat A to be conveyed into the settling chamber 10 and through the instrumentality of the filter 11 the liquid contained in the tailings from the valve 31 will be admitted to the chamber 9 of the vat 1, while the ore carried in suspension by the liquid will be deposited in the chamber 10, it being apparent that the solution when passed through the screen 11 will be reconditioned to bring it back to a clarified state to be used again in the agitating vat A. The exhausted ore after having been treated for extraction is removed from the settling vat in any suitable manner, preferably by the use of a sand pump (not shown) or by any other mechanical means which excludes the removal of the liquid reagent, thus confining the loss of reagent to that which is carried out in the form of a moisture contained in the pulp.

By reason of the formation of the propeller blades 19 of the agitator, when the same is in operation, a suction is created above the position of such blades which has a tendency to sink all mineral particles which might have otherwise a tendency to float on the surface of the solution due to the surface tension of the solution used. The angle of the shaft 18 of the agitator with relation to the angle of the vat is such as to create a downward movement of the solution on the side of the vat where the propeller shaft is located and an outward motion of the solution in the opposite side of the vat, thus keeping the solution with its suspended material in a rapid state of circulation in the vat A in order that the cathode in the bottom of the vat will be continuously bombarded with the mineral particles which are in a state of suspension in such solution.

Included in the electric circuit for the cathode and anode is an ammeter 33 and a rheostat 34, respectively, these being mounted directly on the vat A, thus making it possible to measure and control the current density used in the extraction process.

It is, of course, understood that the chemical reagents, as well as the electric currents, used with the apparatus in amalgamation and separation by the process are many and must be changed in order to bring about a satisfactory extraction of the desired metal or metals from each specific type or variety of ore of which its chemical or mechanical structure may warrant and the principles of using chemical reagents are to make the suspended solution in the vat an electrolyte, so that the metals in the solution will assume a positive electrical charge from the anode

and thus be passed to the cathode or to bring about a complete or partial chemical change in the ore under treatment, or to dissolve partially or completely the metals and convert them into 5 soluble electrolyte salts so that they may be precipitated at the cathode by the electrical current, or to dissolve undesirable metals and make them non-electrolytes so that they will not interfere with the completion of the process. The specific 10 reagents for the leaching of the metals and the formation of electrolyte salts that they may be precipitated at the cathode by the electric current may be potassium hydroxide; potassium chloride; ammonium hydroxide; sulphuric acid; 15 hydrochloric acid; nitric acid; potassium nitrate or sodium nitrate; potassium bichromate; cyanide potassium or potassium sodium and calcium; barium hydroxide; calcium hydroxide and potassium carbonate or calcium carbonate or sodium 20 carbonate.

A reagent may be used to counteract an undesirable condition existing in the ore, such as a strong acidity or alkalinity that may be unfavorable and by the addition of a counteractor bring 25 about the desired condition for the extraction of the metal or metals. This reagent should be called a sizer or conditioner which could be used as an electrolyte or just bring the ore pulp to a neutral condition and the addition of a beneficial 30 reagent to bring the conductivity of the solution to the desired point.

In Figure 4 of the drawings there is shown a slight modification of the apparatus wherein the vat B, at its lower point, has fitted therein an 35 auger 35 having the extended shaft 36 for attachment to a mechanical drive for the rotation thereof and this auger is used for the discharge of concentrates or mercury as may be within the lowermost portion of the vat B, in event that 40 the vat is used as a continuous type concentrator, as will be clearly apparent, the auger housing 37 being formed with a downwardly directed discharge spout 38 for communication with the lowermost vat of the said apparatus.

45 The V shape of the vat utilized in the process has an important bearing not only upon the recovery of desired mineral but also from a standpoint of discharging tailings. The position of the propeller with its downward motion creates

a circulation of the mass or material under treatment on the side that the propeller is located and an upward movement on the opposite slope. It will be noted that the tailings discharge outlet is located in the approximate center of this 5 circulating mass of material. This is very important where mercury is being used as a cathode because if the discharge outlet were located in the propeller slip stream, there would be a tendency to carry over mercury in the discharged tailings. 10 Another important feature is the fact that in an ore that carries mineral in a finely divided state, it is absolutely essential to have this circulating action of the entire mass under treatment to prevent accidental flotation of the mineral particles 15 on the surface of the solution in use in the vat. So it becomes quite evident from the above that the particular shape of the vat is quite important so far as the entire process is concerned.

What is claimed is:

An apparatus of the kind described comprising a downwardly tapered vat closed at its lowermost smaller end and open at its top for receiving comminuted ore and a solution, bearings fixed to the side wall of said vat at the open top thereof, 25 a rotatable shaft journaled in said bearings in close parallel relation to the side wall of said vat and having an agitator head located close to the bottom end of the vat to be deeply submerged in the solution therein for causing a continuous un- 30 restricted down flow of the solution in the direc- 35 tion of the lowermost end of said vat and a circu- 40 lation in an upward direction at the side of the vat remote from said head, a tray beneath the vat and having a vertical partition dividing it 45 into independent compartments, a screen associated with the partition at the upper edge of the latter, a pump operating in one of the compartments for transferring substance therefrom into the vat, a mercurial pocket formed at the lowermost end of the vat and containing mercury, a drain from said pocket, an anode fixed to the side of the vat interiorly thereof and removed from the level of the mercury in the pocket, and a lead from the vat to the other compartment 45

MARTIN W. KROLL.